

# UNITED STATES PATENT OFFICE.

WILLIAM R. VEAZEY, OF CLEVELAND, OHIO, ASSIGNOR TO THE DOW CHEMICAL COMPANY, OF MIDLAND, MICHIGAN, A CORPORATION OF MICHIGAN.

## MAGNESIUM ALLOY.

1,334,193.

Specification of Letters Patent. Patented Mar. 16, 1920.

No Drawing.

Application filed October 10, 1918. Serial No. 257,564.

To all whom it may concern:

Be it known that I, WILLIAM R. VEAZEY, a citizen of the United States, and a resident of Cleveland, county of Cuyahoga, and State of Ohio, have invented a new and useful Improvement in Magnesium Alloys, of which the following is a specification, the principle of the invention being herein explained and the best mode in which I have contemplated applying that principle, so as to distinguish it from other inventions.

Alloys of copper with magnesium are known, but so far as I am aware it has never been heretofore attempted to include manganese as an additional element, any more than to directly alloy manganese and magnesium. Possibly one reason for this has been the difficulty experienced in fusing together the two last named metals, due to the fact that temperatures above the boiling point of magnesium are involved. By the present improved method, however, I have found it possible to produce alloys of all three metals, the resulting product possessing distinctive and highly desirable properties which indicate a wide field of usefulness.

The invention, then, consists of the new product, consisting of an alloy of the metals in question, together with the steps involved in the making of such alloy, hereinafter fully described and particularly set forth in the claims. The following description, it will be understood, thus sets forth but one of the various ways in which the invention may be carried out.

I have found that a relatively very small amount of copper, and a still smaller amount of manganese, need to be added to the magnesium in order to materially affect its properties. Thus the addition of such alloy metals in an amount aggregating not to exceed one (1) per cent., will give a product having a much finer texture than either magnesium alone, or an alloy containing manganese and magnesium, without any considerable increase in specific gravity over that of the magnesium, while such alloy is very much stronger under all the usual tests, and furthermore constitutes an excellent bearing metal.

As an example of my new alloy, I give the following proportions, viz., magnesium 99 per cent., copper  $\frac{1}{10}$  per cent. and manganese  $\frac{4}{10}$  per cent. This alloy has a specific

gravity of approximately 1.8 and under test shows a yielding point of ten thousand (10,000) pounds to the square inch, and an ultimate strength of nineteen thousand (19,000) pounds, with a reduction in area, 60 after elongation, not to exceed six (6) per cent. A bar of the alloy, when struck, gives forth a distinct bell-like tone, in contradistinction to pure magnesium, which sounds 65 dull, like a stick of wood. Such alloy, as indicated above, has also been found to stand up exceedingly well as a bearing metal. Thus a bearing of such metal, when subjected to two hundred and fifteen (215) pounds pressure to the square inch, calculated on the 70 projected area of the bearing, and lubricated in the ordinary manner from an oil cup (i. e. not running in an oil bath), showed a maximum temperature of only eighteen degrees centigrade above that of the room. 75

To make my improved alloy, the proper amount of copper is first added to the magnesium, such copper going in without difficulty, as its melting temperature is relatively low, alloys of copper with magnesium 80 being already known. The manganese is then added in the form of anhydrous manganese chlorid, the magnesium-copper mixture being first melted in a suitable crucible with a flux, for example, of magnesium 85 chlorid and sodium chlorid. The manganese chlorid is thereupon placed directly on the mass of previously molten metal, where it melts, and if left to itself runs over the surface of the mass, and may be thoroughly 90 stirred into such mass. The final alloy may be conveniently removed in molten state from the crucible, by means of an ordinary ladle, and cast into bars or other such shapes as may be desired. The amount of 95 manganese derived from any given quantity of the chlorid is about forty-four (44) per cent., but some of this is apparently lost in the reaction; at least less than the theoretical amount of such manganese appears present in the final alloy. However, by properly calculating the amount of chlorid added, an alloy containing the desired proportion (e. g.  $\frac{4}{10}$  per cent. as in the illustration cited) may 100 be obtained.

While it is preferred, as indicated by the above description, to add the copper first to the metallic magnesium, in making my improved alloy, it is entirely possible to add the manganese chlorid first, thus making a 110

mixture, or perhaps an alloy of manganese and magnesium, to which the metallic copper is subsequently added.

Other modes of applying the principle 5 of my invention may be employed instead of the one explained, change being made as regards the composition and method herein disclosed, provided the ingredients or steps stated by any of the following 10 claims or the equivalent of such stated ingredients or steps be employed.

I therefore particularly point out and distinctly claim as my invention:—

1. As a new product, an alloy of manganese and copper with magnesium, the manganese and copper aggregating a relatively small per cent. of the total.

2. As a new product, an alloy of manganese and copper with magnesium, the manganese and copper aggregating approximately one (1) per cent. of the total.

3. As a new product, an alloy of manganese and copper with magnesium, the manganese and copper aggregating approximately one (1) per cent. of the total, and slightly more copper than manganese being used.

4. As a new product, an alloy of approximately four-tenths ( $\frac{4}{10}$ ) per cent. copper, six-tenths ( $\frac{6}{10}$ ) per cent. manganese, and ninety-nine (99) per cent. magnesium.

5. The method of making a copper-manganese-magnesium alloy, which consists in first inter-fusing the desired amount of copper with the magnesium, and then adding the desired amount of manganese.

6. The method of making a copper-manganese-magnesium alloy, which consists in first inter-fusing the desired amount of copper with the magnesium, and then adding the desired amount of manganese, the copper being added in the form of the

metal direct, and the manganese in the form of a reducible compound to the copper-magnesium alloy thus preliminarily formed.

7. The method of making a copper-manganese-magnesium alloy, which consists in first inter-fusing the desired amount of copper with the magnesium, and then adding the desired amount of manganese, the copper being added in the form of the metal direct, and the manganese in the form of manganese chlorid to the copper-magnesium alloy thus preliminarily formed.

8. The method of making a copper-manganese-magnesium alloy, which consists in first inter-fusing the desired amount of copper with the magnesium, and then adding the desired amount of manganese, the copper being added in the form of the metal direct, and the manganese in the form of anhydrous manganese chlorid to the copper-magnesium alloy thus preliminarily formed.

9. The method of making a copper-manganese-magnesium alloy, which consists in first inter-fusing the desired amount of copper with the magnesium, and then adding the desired amount of manganese, the amount of manganese and copper in the final product aggregating approximately one (1) per cent. of the total.

10. The method of making a copper-manganese-magnesium alloy, which consists in first inter-fusing the desired amount of copper with the magnesium, and then adding the desired amount of manganese, the amount of manganese and copper in the final product respectively equalling approximately four-tenths ( $\frac{4}{10}$ ) per cent. and six-tenths ( $\frac{6}{10}$ ) per cent. of the total.

Signed by me, this 3rd day of October, 1918.

WILLIAM R. VEAZEY.